# EUROPEAN PATENT SPECIFICATION

(11) **EP 4 187 558 B1**
(45) Date of publication and mention of the grant of the patent: **24.07.2024**
(21) Application number: 22206155.8
(22) Date of filing: 08.11.2022
(51) Int. Cl.: H01F 1/01, H01F 1/055, H01F 7/02, H01F 41/02, B22F 1/10

(54) **APPLICATION OF AN ADDITIVE IN A PREPARATION METHOD OF A SAMARIUM-COBALT 2:17 TYPE MAGNET**
ANWENDUNG EINES ADDITIVS IN EINEM HERSTELLUNGSVERFAHREN FÜR SAMARIUM-KOBALT-2:17-TYP-MAGNET
APPLICATION D'UN ADDITIF DANS UN PROCÉDÉ DE PRÉPARATION D'AIMANT DE TYPE SAMARIUM-COBALT 2:17

(30) Priority: 30.11.2021 CN 202111444382
(43) Date of publication of application: 31.05.2023
(73) Proprietor: Fujian Changting Zorr Technology Co., Ltd., Chanting County Longyan, Fujian 366300 (CN); Xiamen Tungsten Co., Ltd., Xiamen, Fujian 361000 (CN)
(72) Inventor: FU, Zhongwei, Longyan, Fujian 366300 (CN); OUYANG, Fuzhong, Longyan, Fujian 366300 (CN); ZHANG, Chang, Longyan, Fujian 366300 (CN); WU, Maolin, Longyan, Fujian 366300 (CN); WANG, Guoxiong, Longyan, Fujian 366300 (CN); SHI, Dawei, Longyan, Fujian 366300 (CN)
(74) Representative: karo IP

(56) References cited:
- CN-A- 111 145 973
- CN-A- 111 370 191
- CN-A- 113 593 882
- US-A1- 2020 243 232
- US-A1- 2020 243 233
- US-A1- 2021 079 248

## Description

### Field of the Invention

The present invention relates to the use of an additive in the preparation of a samarium-cobalt 2: 17 type magnet and a preparation method thereof.

### Background of the Invention

The phenomenon of copper depletion at grain boundaries commonly occurs in Sm₂Co₁₇ permanent magnet materials (also referred to as samarium-cobalt 2: 17 type magnets) and has become an obstacle for the improvement of properties, especially the squareness, of the Sm₂Co₁₇ permanent magnet materials. The grain boundary structure with copper depletion has a weak domain wall pinning field, which can easily form a reversal magnetization center during demagnetization, thereby reducing the coercivity, squareness, and magnetic energy product of magnets.

The current practice is to improve the phenomenon of copper depletion at grain boundaries by adding micro or nano copper or copper oxide powder directly to jet-milled powder. For example, CN111145973A discloses a preparation method of a magnet containing a Cu grain boundary phase, in which CuO powder is mixed with samarium-cobalt powder, and the mixture is pressed and sintered. Although the method can improve the coercivity and squareness to certain extents, the oversize micro powder and introduction of a nonmagnetic grain boundary phase cause the reduction of remanence. Moreover, the micro powder cannot be uniformly dispersed, so that an achieved effect is limited. In addition, a copper diffusion method for regulating and controlling grain boundaries has also been reported, but this diffusion method is only effective for sheet samples only, so its use is limited.

US 2021/0079248 A1 discloses a molecular ink comprising a flake-less printable composition of 5-75 wt% of bis(2-ethyl-1-hexylamine) copper (II) formate, bis(octylamine) copper (II) formate or tris(octylamine) copper (II) formate; 0.25-10 wt % of a polymeric binder; and, balance of at least one organic solvent, all weights based on total weight of the composition, wherein the binder comprises ethyl cellulose, and the ethyl cellulose has an average weight molecular weight in a range of 60,000-95,000 g/mol and a bimodal molecular weight distribution.

### Summary of the Invention

In order to solve the defect that in the prior art, the coercivity and squareness are only improved to limited extents and the remanence may be reduced when overcoming the problem of poor magnetic properties, especially low squareness, of Sm₂Co₁₇ permanent magnet materials caused by the phenomenon of copper depletion at grain boundaries, the present invention provides the use of an additive in the preparation of a samarium-cobalt 2: 17 type magnet and a preparation method thereof. The preparation method of a Sm₂Co₁₇ permanent magnet of the present invention can greatly eliminate adverse effects brought by the phenomenon of copper depletion at grain boundaries without reducing the remanence, thereby improving the coercivity, squareness, and magnetic energy product of products.

The present invention adopts the following technical solutions to solve the above technical problem.

The present invention provides the use of an additive, which includes the following components by mass percentage: 20-30% of organocopper complex, 0.5-1% of plasticizer, and an organic solvent, and the sum of the mass percentages of the components is 100%,
wherein the organocopper complex is an oil-soluble substance, the mass percentage of Cu in the organocopper complex is greater than 10%, and the organocopper complex contains a polar group and/or an alkyl chain having more than 3 C atoms,
in the preparation of a samarium-cobalt 2: 17 type magnet.

In the present invention, the organocopper complex may be a conventional oil-soluble organocopper complex in the art, for example, may be completely dissolved in an inert solvent such as toluene and mineral oil. The inert solvent generally refers to a solvent that does not chemically react with the organocopper complex.

Preferably, the polar group in the organocopper complex is one or more of a hydroxyl group, a carboxyl group, an amino group, an ester group, and an amide group.

The alkyl chain in the organocopper complex may be a saturated alkyl chain or an unsaturated alkyl chain, and the alkyl chain may be a straight chain or a branched chain.

Preferably, the organocopper complex is one or more of a substituted copper carboxylate complex, a copper carboxylate derivative, a copper thiophosphate complex, copper quinoline, copper hydroxyquinoline, copper phthalate, thiodiazole copper, copper acetylacetonate, and copper acetoacetate.

A general formula of the substituted copper carboxylate complex is preferably [RCO₂]₂Cu, where, R is alkyl, alkynyl, cyclo, aryl or heteroaryl; preferably, the substituted copper carboxylate complex is one or more of fatty acid copper having 10 to 22 carbon atoms, copper styrene maleate, copper picolinate, copper 2-pyrazinecarboxylate, copper 2-ethylhexanoate, copper methacrylate, copper thiophene-2-carboxylate, copper methionine, and copper tartrate, and the fatty acid copper having 10 to 22 carbon atoms is preferably one or more of copper oleate, copper linoleate, copper stearate, copper rosinate, copper hexadecanoate, copper palmitate, and copper naphthenate.

The copper carboxylate derivative is preferably a copper thiocarboxylate derivative [R'CS₂]₂Cu or a copper selenocarboxylate derivative [R'CSe₂]₂Cu, where, R' includes alkyl and alkyl derivatives; and preferably, the copper carboxylate derivative is copper N,N-di-n-butyldithiocarbamate (Cu(SC(S)N(C₄H₉)₂)₂) and/or copper N,N-din-butyldiselenocarbamate (Cu(SeC(Se)N(C₄H₉)₂)₂).

The copper thiophosphate complex is preferably a copper complex of a dialkyldithiophosphate, and a general formula of the copper complex of the dialkyldithiophosphate is (RO)₂P(S)SHM, where, R is alkyl or aryl, and M includes monovalent copper and divalent copper (CuDDP for short); and preferably, the copper thiophosphate complex is one or more of copper dihexyldithiophosphate, copper dibutyldithiophosphate, copper-containing antioxidant T541, and copper-containing antioxidant T542. The copper-containing antioxidant T541 and the copper-containing antioxidant T542 can be purchased from the additive factory of Jinzhou Petrochemical Corporation.

Preferably, the grain diameter of the organocopper complex is less than 10 µm.

In the present invention, preferably, the mass percentage of the organocopper complex in the additive is 20%, 22%, 23%, 25%, 27% or 30%.

In the present invention, the plasticizer may be a conventional plasticizer in the art, preferably, the plasticizer is a phthalate and/or epoxidized soybean oil, and more preferably, the plasticizer is one or more of dibutyl phthalate, dioctyl phthalate, and epoxidized soybean oil. Through the cooperation of the usage amount of the plasticizer and other components of the additive, the organocopper complex can be uniformly dispersed on the surface of powder, agglomeration between the organocopper complexes can be prevented, Cu is uniformly distributed at grain boundaries after the organocopper complex is decomposed, the grain boundary Cu concentration is basically equivalent to the intragranular Cu concentration, and the phenomenon of copper depletion at grain boundaries is avoided.

In the present invention, preferably, the mass percentage of the plasticizer in the additive is 0.5%, 0.8% or 1%.

In the present invention, the organic solvent may be a conventional organic solvent in the art, preferably, the organic solvent is one or more of acetone, toluene, mineral oil, methyl acetate, 120# solvent oil, isooctane, isopropanol, chloroform, and methyl methacrylate, and more preferably, the organic solvent is one or more of 120# solvent oil, toluene, mineral oil, acetone, isooctane, and isopropanol, such as 120# solvent oil, toluene, mineral oil, a mixed solvent of isooctane and isopropanol, and a mixed solvent of acetone and isopropanol.

In the present invention, preferably, the mass percentage of the organic solvent in the additive is 69-79.5%.

In the present invention, preferably, the additive is composed of 20-30% of organocopper complex, 0.5-1% of plasticizer, and 69-79.5% of organic solvent.

The present invention also provides a preparation method of the above additive, which includes the following step:
mixing the organocopper complex, the plasticizer, and the organic solvent.

The present invention provides the use of the above additive in the preparation of a samarium-cobalt magnet. The additive has the effects of lubricating and regulating and controlling grain boundaries of samarium-cobalt magnets, can improve the phenomenon of copper depletion at grain boundaries, and improve the remanence, coercivity, and squareness of magnets.

The present invention also provides a preparation method of a samarium-cobalt 2: 17 type magnet, which includes the following steps: mixing samarium-cobalt magnet alloy powder with the above additive, shaping, sintering, and aging.

The mass percentage of Cu in the organocopper complex in the samarium-cobalt magnet alloy powder is 0.1-0.2%.

In the present invention, preferably, raw materials of the samarium-cobalt magnet alloy powder include Sm, Cu, Fe, Zr, and Co.

Preferably, the mass percentage of Sm in the raw materials of the samarium-cobalt magnet alloy powder is 24-26% such as 24%, 25.5%, and 26%.

Preferably, the mass percentage of Cu in the raw materials of the samarium-cobalt magnet alloy powder is 4-6% such as 4%, 5.5%, and 6%.

Preferably, the mass percentage of Fe in the raw materials of the samarium-cobalt magnet alloy powder is 10-20% such as 10%, 17%, 19%, and 20%.

Preferably, the mass percentage of Zr in the raw materials of the samarium-cobalt magnet alloy powder is 2.0-4% such as 2.0%, 3.5%, and 4%.

Preferably, the mass percentage of Co in the raw materials of the samarium-cobalt magnet alloy powder is 45-60% such as 46%, 48%, 51.5%, and 56%.

In a preferred embodiment of the present invention, the samarium-cobalt magnet alloy powder is composed of 24% of Sm, 4% of Cu, 17% of Fe, 3.5% of Zr, 51.5% of Co.

In a preferred embodiment of the present invention, the samarium-cobalt magnet alloy powder is composed of 25.5% of Sm, 5.5% of Cu, 19% of Fe, 2% of Zr, and 48% of Co.

In a preferred embodiment of the present invention, the samarium-cobalt magnet alloy powder is composed of 26% of Sm, 4% of Cu, 10% of Fe, 4% of Zr, and 56% of Co.

In a preferred embodiment of the present invention, the samarium-cobalt magnet alloy powder is composed of 24% of Sm, 6% of Cu, 20% of Fe, 4% of Zr, and 46% of Co.

Preferably, the samarium-cobalt magnet alloy powder is obtained by smelting and crushing the raw materials of the samarium-cobalt magnet alloy powder.

Preferably, the smelting is performed by melt-spinning, centrifugal casting or ingot casting.

Preferably, the crushing includes coarse crushing, secondary crushing, and fine crushing, wherein the coarse crushing is preferably Jaw crushing, the secondary crushing is preferably disc milling or crushing with an intermediate crusher, and the fine crushing is preferably jet milling or ball milling.

Preferably, the grain diameter D50 of the samarium-cobalt magnet alloy powder is 4-6 µm.

Preferably, the samarium-cobalt magnet alloy powder is mixed with the additive, and the mixture is dried to remove most of the solvent, shaped, sintered, and aged. The drying is preferably placing the powder in a dryer and drying at 80°C for 5-10 h such as 5 h, 6h, 6.5 h, 7h, 7.5 h, 8 h, and 10 h.

In the present invention, preferably, the mass percentage of Cu in the organocopper complex in the samarium-cobalt magnet alloy powder is 0.1%, 0.12%, 0.14%, 0.16%, 0.18% or 0.2%, and an addition amount of the additive is determined by the copper content in a selected substance and the solution concentration.

In a preferred embodiment of the present invention, the additive is composed of 25% of copper naphthenate, 0.50% of epoxidized soybean oil, and 74.5% of 120# solvent oil; and the mass percentage of the additive in the samarium-cobalt magnet alloy powder is preferably 2.5%.

In a preferred embodiment of the present invention, the additive is composed of 30% of copper oleate, 0.50% of epoxidized soybean oil, and 69.5% of 120# solvent oil; and the mass percentage of the additive in the samarium-cobalt magnet alloy powder is preferably 3.3%.

In a preferred embodiment of the present invention, the additive is composed of 30% of copper hexadecanoate, 0.50% of dibutyl phthalate, and 69.5% of 120# solvent oil; and the mass percentage of the additive in the samarium-cobalt magnet alloy powder is preferably 3.6%.

In a preferred embodiment of the present invention, the additive is composed of 27% of copper N,N-di-n-butyldithiocarbamate, 0.50% of dibutyl phthalate, and 72.5% of toluene; and the mass percentage of the additive in the samarium-cobalt magnet alloy powder is preferably 3.3%.

In a preferred embodiment of the present invention, the additive is composed of 25% of copper dihexyldithiophosphate, 0.80% of epoxidized soybean oil, and 74.2% of toluene; and the mass percentage of the additive in the samarium-cobalt magnet alloy powder is preferably 3.4%.

In a preferred embodiment of the present invention, the additive is composed of 22% of copper dibutyldithiophosphate, 0.80% of dioctyl phthalate, and 77.2% of mineral oil; and the mass percentage of the additive in the samarium-cobalt magnet alloy powder is preferably 2.4%.

In a preferred embodiment of the present invention, the additive is composed of 23% of T541, 0.80% of dioctyl phthalate, and 76.2% of mineral oil; and the mass percentage of the additive in the samarium-cobalt magnet alloy powder is preferably 3.5%.

In a preferred embodiment of the present invention, the additive is composed of 20% of copper acetylacetonate, 1% of epoxidized soybean oil, 40% of isooctane, and 39% of isopropanol; and the mass percentage of the additive in the samarium-cobalt magnet alloy powder is preferably 3.7%.

In a preferred embodiment of the present invention, the additive is composed of 23% of copper acetoacetate, 1% of epoxidized soybean oil, 40% of acetone, and 36% of isopropanol; and the mass percentage of the additive in the samarium-cobalt magnet alloy powder is preferably 4.4%.

In a preferred embodiment of the present invention, the additive is composed of 20% of copper hexadecanoate, 1% of epoxidized soybean oil, 40% of isooctane, and 39% of isopropanol; and the mass percentage of the additive in the samarium-cobalt magnet alloy powder is preferably 8.1%.

In a preferred embodiment of the present invention, the additive is composed of 23% of copper oleate, 1% of epoxidized soybean oil, 40% of acetone, and 36% of isopropanol; and the mass percentage of the additive in the samarium-cobalt magnet alloy powder is preferably 8.7%.

In the present invention, the shaping operation and conditions may be conventional in the art, and preferably, the shaping is oriented compression shaping performed in a static magnetic field.

Preferably, the magnetic field strength B for shaping is 1.5-2 T.

In the present invention, the sintering operation and conditions are conventional in the art.

Preferably, the sintering is performed in an inert atmosphere.

Preferably, the sintering temperature is 1200-1220°C such as 1200°C, 1210°C, 1215°C, and 1220°C.

Preferably, the sintering time is 1-5 h such as 1 h, 3 h, 4 h, and 5 h.

In the present invention, preferably, solution treatment is performed after sintering.

Preferably, the solution treatment temperature is 1140-1190°C such as 1140°C, 1150°C, 1160°C, and 1190°C.

Preferably, the solution treatment time is 5-40 h such as 5 h, 20 h, 35 h, and 40 h.

In the present invention, the aging operation and conditions are conventional in the art.

Preferably, the aging is keeping at 800-900°C (e.g., 810°C, 840°C, 860°C, and 900°C) for 5-20 h (e.g., 5 h, 15 h, and 20 h), cooling to 400°C, and keeping for 5-10 h (e.g., 5 h, 6 h, 7 h, and 10 h).

Preferably, the cooling is performed at a rate of 0.7°C/min.

On the basis of conforming to common knowledge in the art, the above preferred conditions can be combined arbitrarily to obtain preferred embodiments of the present invention.

The reagents and materials used in the present invention are all commercially available.

The present invention has the following positive progressive effects.

The method of using an additive containing an organocopper complex to regulate and control grain boundaries is easy to operate, does not require extra process procedures, and does not have special requirements for the shape and size of a product, so it is suitable for batch production. Compared to a product prepared by the conventional method, a finally obtained product has basically equivalent remanence, the coercivity is increased by 5-10 kOe, Hk is increased by 1-4 kOe, and the squareness can reach 60-75%.

### Brief Description of the Drawings

Fig. 1 is a comparison curve diagram of magnetic properties of samples of Example 4 and Contrast 4;
Fig. 2 is a scanning image of a distributive area of Cu at grain boundaries of the sample of Contrast 4;
Fig. 3 is a scanning image of a distributive area of Cu at grain boundaries of the sample of Example 4;
Fig. 4 is a line scanning image of the grain boundary Cu concentration in the sample of Contrast 4; and
Fig. 5 is a line scanning image of the grain boundary Cu concentration in the sample of Example 4.

### Detailed Description of the Embodiments

The present invention will be further described below with reference to examples, but the present invention is not limited to the range of the examples. Experimental methods that do not indicate specific conditions in the following examples follow conventional methods and conditions or product manuals.

### Example 1

(1) Raw materials of samarium-cobalt magnet alloy powder shown in Table 1 were smelted and crushed to obtain samarium-cobalt magnet alloy powder, and the grain diameter D50 of the samarium-cobalt magnet alloy powder was 4-6 µm.

The smelting was performed by melt-spinning, centrifugal casting or ingot casting; the crushing was coarse crushing, secondary crushing, and fine crushing that were performed in sequence, the coarse crushing was Jaw crushing, the secondary crushing was disc milling or crushing with an intermediate crusher; and the fine crushing was jet milling.

(2) The samarium-cobalt magnet alloy powder obtained at step (1) was mixed with an additive shown in Table 2, and the mixture was dried by using a dryer in a 99.99% N₂ atmosphere at 80°C for a period of time shown in Table 1. Then, the mixture was shaped, sintered, and aged. An addition amount of the additive was determined by a set effective addition amount of Cu (the mass percentage of Cu in the organocopper complex in the samarium-cobalt magnet alloy powder) and the solution concentration, see Table 1.

The fine crushing was jet milling or ball milling. Oriented compression shaping was performed in a static magnetic field. The magnetic field strength for shaping, the sintering temperature and time, solution treatment temperature and time, and aging operation are shown in Table 3. The cooling in the aging was performed at a rate of 0.7°C/min.

**Table 1 Raw materials of samarium-cobalt magnet alloy powders of examples and contrasts**

| | Samarium-cobalt magnet alloy powder (mass percentage) | | | | | Mass percentage of additive in samarium-cobalt magnet alloy powder / % | Drying time / h |
|---|---|---|---|---|---|---|---|
| | Sm | Cu | Fe | Zr | Co | | |
| Example 1 | 24 | 4 | 17 | 3.5 | balance | 2.5 | 5 |
| Example 2 | 24 | 4 | 17 | 3.5 | balance | 3.3 | 6 |
| Example 3 | 24 | 4 | 17 | 3.5 | balance | 3.6 | 7.5 |
| Example 4 | 25.5 | 5.5 | 19 | 2 | balance | 3.3 | 6 |
| Example 5 | 25.5 | 5.5 | 19 | 2 | balance | 3.4 | 6.5 |
| Example 6 | 25.5 | 5.5 | 19 | 2 | balance | 2.4 | 5 |
| Example 7 | 26 | 4 | 10 | 4 | balance | 3.5 | 7 |
| Example 8 | 26 | 4 | 10 | 4 | balance | 3.7 | 8 |
| Example 9 | 24 | 6 | 20 | 4 | balance | 4.4 | 10 |
| Example 10 | 26 | 4 | 10 | 4 | balance | 8.1 | 8 |
| Example 11 | 24 | 6 | 20 | 4 | balance | 8.7 | 10 |
| Contrast 1 | 24 | 4 | 17 | 3.5 | balance | 0.4 | 5 |
| Contrast 2 | 24 | 4 | 17 | 3.5 | balance | 0.3 | 6 |
| Contrast 3 | 24 | 4 | 17 | 3.5 | balance | 0.4 | 7.5 |
| Contrast 4 | 25.5 | 5.5 | 19 | 2 | balance | 0.4 | 6 |
| Contrast 5 | 25.5 | 5.5 | 19 | 2 | balance | 0.14 | 6.5 |
| Contrast 6 | 25.5 | 5.5 | 19 | 2 | balance | 0.14 | 5 |
| Contrast 7 | 26 | 4 | 10 | 4 | balance | 0.16 | 7 |
| Contrast 8 | 26 | 4 | 10 | 4 | balance | 1.6 | 8 |
| Contrast 9 | 24 | 6 | 20 | 4 | balance | 11 | 10 |
| Contrast 10 | 24 | 6 | 20 | 4 | balance | 4.4 | 10 |

**Table 2 Components of additives of examples and contrasts and mass percentages thereof**

| | Organocopper complex | | | Plasticizer | | Solvent | | Effecti ve additio n amount of Cu /% |
|---|---|---|---|---|---|---|---|---|
| | Variety | Cu conte nt/% | Usage amou nt/% | Variety | Usage amou nt/% | Variety | Usage amount /% | |
| Examp le 1 | Copper naphthenate | 15.7 | 25 | Epoxidiz ed soybean oil | 0.5 | 120# solvent oil | balance | 0.1 |
| Examp le 2 | Copper oleate | 10 | 30 | Epoxidiz ed soybean oil | 0.5 | 120# solvent oil | balance | 0.1 |
| Examp le 3 | Copper hexadecanoate | 11.08 | 30 | Dibutyl phthalate | 0.5 | 120# solvent oil | balance | 0.12 |
| Examp le 4 | Copper N,N-di-n-butyldithiocarbama te | 13.5 | 27 | Dibutyl phthalate | 0.5 | Toluene | balance | 0.12 |
| Examp le 5 | Copper dihexyldithiophosp hate | 16.5 | 25 | Epoxidiz ed soybean oil | 0.8 | Toluene | balance | 0.14 |
| Examp le 6 | Copper dibutyldithiophosp hate | 26.2 | 22 | Dioctyl phthalate | 0.8 | Mineral oil | balance | 0.14 |
| Examp le 7 | T541 | about 20 | 23 | Dioctyl phthalate | 0.8 | Mineral oil | balance | 0.16 |
| Examp le 8 | Copper acetylacetonate | 24.3 | 20 | Epoxidiz ed soybean oil | 1 | Isooctane | 40% | 0.18 |
| | | | | | | Isopropanol | balance | |
| Examp le 9 | Copper acetoacetate | 19.7 | 23 | Epoxidiz ed soybean oil | 1 | Acetone | 40% | 0.2 |
| | | | | | | Isopropanol | balance | |
| Examp le 10 | Copper hexadecanoate | 11.08 | 20 | Epoxidiz ed soybean oil | 1 | Isooctane | 40% | 0.18 |
| | | | | | | Isopropanol | balance | |
| Examp le 11 | Copper oleate | 10 | 23 | Epoxidiz ed soybean oil | 1 | Acetone | 40% | 0.2 |
| | | | | | | Isopropanol | balance | |
| Contra st 1 | conventional lubricant (butyl oleate) | 0 | 25 | / | / | 120# solvent oil | balance | 0 |
| Contra st 2 | conventional lubricant (butyl oleate) | 0 | 30 | / | / | 120# solvent oil | balance | 0 |
| Contra st 3 | conventional lubricant (methyl decanoate) | 0 | 30 | / | / | 120# solvent oil | balance | 0 |
| Contra st 4 | conventional lubricant (poly(α-olefin)) | 0 | 27 | / | / | Toluene | balance | 0 |
| Contra st 5 | Copper dihexyldithiophosp hate | 16.5 | / | / | / | / | / | 0.14 |
| Contra st 6 | Copper dibutyldithiophosp hate | 26.2 | / | / | / | / | / | 0.14 |
| Contra st 7 | T541 | about 20 | / | / | / | / | / | 0.16 |
| Contra st 8 | Copper acetylacetonate | 24.3 | 13 | Epoxidiz ed soybean oil | 1 | Isooctane | 40% | 0.05 |
| | | | | | | Isopropanol | balance | |
| Contra st 9 | Copper acetoacetate | 19.7 | 23 | Epoxidiz ed soybean oil | 1 | Acetone | 40% | 0.5 |
| | | | | | | Isopropa nol | balan ce | |
| Contra st 10 | Copper acetoacetate | 19.7 | 23 | / | / | Acetone | 40% | 0.2 |
| | | | | | | Isopropanol | balance | |

**Table 3 Parameters of shaping, sintering, solution treatment, and aging of examples and contrasts**

| | Magnetic field strength for shaping | Sintering Temperature | Time | Solution Treatment Temperature | Time | Aging |
|---|---|---|---|---|---|---|
| Example 1 | 1.5T | 1210 | 3 | 1160 | 20 | keep at 840°C for 20 h, cool to 400°C, and keep for 6 h |
| Example 2 | 1.5T | 1210 | 3 | 1160 | 20 | keep at 840°C for 20 h, cool to 400°C, and keep for 6 h |
| Example 3 | 1.5T | 1210 | 3 | 1160 | 20 | keep at 840°C for 20 h, cool to 400°C, and keep for 6 h |
| Example 4 | 1.5T | 1215 | 4 | 1150 | 35 | keep at 860°C for 15 h, cool to 400°C, and keep for 7 h |
| Example 5 | 1.5T | 1215 | 4 | 1150 | 35 | keep at 860°C for 15 h, cool to 400°C, and keep for 7 h |
| Example 6 | 1.5T | 1215 | 4 | 1150 | 35 | keep at 860°C for 15 h, cool to 400°C, and keep for 7 h |
| Example 7 | 2.0T | 1200 | 1 | 1190 | 5 | keep at 810°C for 20 h, cool to 400°C, and keep for 10 h |
| Example 8 | 2.0T | 1200 | 1 | 1190 | 5 | keep at 810°C for 20 h, cool to 400°C, and keep for 10 h |
| Example 9 | 2.0T | 1220 | 5 | 1140 | 40 | keep at 900°C for 5 h, cool to 400°C, and keep for 5 h |
| Example 10 | 2.0T | 1200 | 1 | 1190 | 5 | keep at 810°C for 20 h, cool to 400°C, and keep for 10 h |
| Example 11 | 2.0T | 1220 | 5 | 1140 | 40 | keep at 900°C for 5 h, cool to 400°C, and keep for 5 h |
| Contrast 1 | 1.5T | 1210 | 3 | 1160 | 20 | keep at 840°C for 20 h, cool to 400°C, and keep for 6 h |
| Contrast 2 | 1.5T | 1210 | 3 | 1160 | 20 | keep at 840°C for 20 h, cool to 400°C, and keep for 6 h |
| Contrast 3 | 1.5T | 1210 | 3 | 1160 | 20 | keep at 840°C for 20 h, cool to 400°C, and keep for 6 h |
| Contrast 4 | 1.5T | 1215 | 4 | 1150 | 35 | keep at 860°C for 15 h, cool to 400°C, and keep for 7 h |
| Contrast 5 | 1.5T | 1215 | 4 | 1150 | 35 | keep at 860°C for 15 h, cool to 400°C, and keep for 7 h |
| Contrast 6 | 1.5T | 1215 | 4 | 1150 | 35 | keep at 860°C for 15 h, cool to 400°C, and keep for 7 h |
| Contrast 7 | 2.0T | 1200 | 1 | 1190 | 5 | keep at 810°C for 20 h, cool to 400°C, and keep for 10 h |
| Contrast 8 | 2.0T | 1200 | 1 | 1190 | 5 | keep at 810°C for 20 h, cool to 400°C, and keep for 10 h |
| Contrast 9 | 2.0T | 1220 | 5 | 1140 | 40 | keep at 900°C for 5 h, cool to 400°C, and keep for 5 h |
| Contrast 10 | 2.0T | 1220 | 5 | 1140 | 40 | keep at 900°C for 5 h, cool to 400°C, and keep for 5 h |

### Examples 2 to 11 and Contrasts 1 to 10

Samarium-cobalt magnet alloy powder raw materials and additives were prepared according to the formulas shown in Tables 1 and 2, and other process conditions were the same as those in Example 1 in addition to the operation parameters shown in Table 3.

The additives of Contrasts 1 to 4 contained a lubricant and an organic solvent only; the additives of Contrasts 5 to 7 contained an organocopper complex only; and the additive of Contrast 10 contained an organocopper complex and an organic solvent only.

### Effect Example

Magnetic properties, i.e., the remanence Br, the intrinsic coercivity Hcj, a knee point Hk, the squareness Hk/Hcj, and the maximum magnetic energy product (BH)max, of the examples and the contrasts of the present invention were detected by using a pulse magnetic field meter (PFM). Results are shown in Table 4.

**Table 4 Data of magnetic properties of examples and contrasts**

| | Br (kGs) | Hcj (kOe) | Hk (kOe) | Hk/Hcj (%) | BHmax (MGOe) |
|---|---|---|---|---|---|
| Example 1 | 11.52 | 32.44 | 19.47 | 60.00 | 32.88 |
| Example 2 | 11.53 | 33.01 | 19.89 | 60.25 | 32.92 |
| Example 3 | 11.60 | 34.56 | 21.55 | 62.36 | 33.02 |
| Example 4 | 11.94 | 26.23 | 16.98 | 64.74 | 33.14 |
| Example 5 | 11.93 | 26.85 | 17.79 | 66.26 | 33.25 |
| Example 6 | 11.93 | 27.88 | 18.56 | 66.57 | 33.52 |
| Example 7 | 10.04 | 29.88 | 21.51 | 72 | 24.55 |
| Example 8 | 10.05 | 32.25 | 23.86 | 74 | 25.24 |
| Example 9 | 12.16 | 27.53 | 20.65 | 75 | 34.71 |
| Example 10 | 10.02 | 30.25 | 20.82 | 68.8 | 24.84 |
| Example 11 | 12.11 | 25.93 | 18.75 | 72.3 | 34.33 |
| Contrast 1 | 11.48 | 23.88 | 14.52 | 60.80 | 31.52 |
| Contrast 2 | 11.49 | 23.91 | 14.66 | 61.31 | 31.61 |
| Contrast 3 | 11.52 | 24.62 | 14.63 | 59.42 | 31.58 |
| Contrast 4 | 11.93 | 22.56 | 12.20 | 54.08 | 33.02 |
| Contrast 5 | 11.86 | 24.21 | 12.18 | 50.31 | 32.84 |
| Contrast 6 | 11.87 | 24.56 | 12.14 | 49.43 | 32.86 |
| Contrast 7 | 9.98 | 21.89 | 12.24 | 55.92 | 24.01 |
| Contrast 8 | 9.84 | 24.15 | 13.32 | 55.16 | 23.71 |
| Contrast 9 | 12.01 | 11.52 | 3.01 | 26.1 | 27.94 |
| Contrast 10 | 12.03 | 21.36 | 11.75 | 55 | 33.21 |

As shown in Fig. 1 to Fig. 5, in the sample of Example 4, Cu is distributed uniformly at grain boundaries, and the grain boundary Cu concentration is basically equivalent to the intragranular Cu concentration, so that the phenomenon of copper depletion at grain boundaries is avoided. With regard to product performance, compared to the samples prepared by the conventional method, the samples of the examples have basically equivalent remanence, the coercivity is increased by 5-10 kOe, Hk is increased by 1-4 kOe, and the squareness can reach 60-75%.

## Claims

1. Use of an additive, **characterized by** comprising the following components by mass percentage: 20-30% of organocopper complex, 0.5-1% of plasticizer, and an organic solvent, the sum of the mass percentages of the components being 100%,
the organocopper complex being an oil-soluble substance, the mass percentage of Cu in the organocopper complex being greater than 10%, the organocopper complex containing a polar group and/or an alkyl chain having more than 3 C atoms,
in the preparation of a samarium-cobalt 2: 17 type magnet.

2. The use according to claim 1, **characterized in that** the additive satisfies one or more of the following conditions:
(1) the polar group in the organocopper complex is one or more of a hydroxyl group, a carboxyl group, an amino group, an ester group, and an amide group;
(2) the organocopper complex is one or more of a substituted copper carboxylate complex, a copper carboxylate derivative, a copper thiophosphate complex, copper quinoline, copper hydroxyquinoline, copper phthalate, thiodiazole copper, copper acetylacetonate, and copper acetoacetate;
a general formula of the substituted copper carboxylate complex is preferably [RCO₂]₂Cu, where, R is alkyl, alkynyl, cyclo, aryl or heteroaryl; preferably, the substituted copper carboxylate complex is one or more of fatty acid copper having 10 to 22 carbon atoms, copper styrene maleate, copper picolinate, copper 2-pyrazinecarboxylate, copper 2-ethylhexanoate, copper methacrylate, copper thiophene-2-carboxylate, copper methionine, and copper tartrate, and the fatty acid copper having 10 to 22 carbon atoms is preferably one or more of copper oleate, copper linoleate, copper stearate, copper rosinate, copper hexadecanoate, copper palmitate, and copper naphthenate;
the copper carboxylate derivative is preferably a copper thiocarboxylate derivative [R'CS₂]₂Cu or a copper selenocarboxylate derivative [R'CSe₂]₂Cu, where, R' comprises alkyl and alkyl derivatives; and preferably, the copper carboxylate derivative is copper N,N-di-n-butyldithiocarbamate and/or copper N,N-di-n-butyldiselenocarbamate;
the copper thiophosphate complex is preferably a copper complex of a dialkyldithiophosphate, and a general formula of the copper complex of the dialkyldithiophosphate is (RO)₂P(S)SHM, where, R is alkyl or aryl, and M comprises monovalent copper and divalent copper; and preferably, the copper thiophosphate complex is one or more of copper dihexyldithiophosphate, copper dibutyldithiophosphate, copper-containing antioxidant T541, and copper-containing antioxidant T542;
(3) the grain diameter of the organocopper complex is less than 10 µm;
(4) the mass percentage of the organocopper complex in the additive is 20%, 22%, 23%, 25%, 27% or 30%;
(6) the plasticizer is a phthalate and/or epoxidized soybean oil, and preferably, the plasticizer is one or more of dibutyl phthalate, dioctyl phthalate, and epoxidized soybean oil;
(7) the mass percentage of the plasticizer in the additive is 0.5%, 0.8% or 1%;
(8) the organic solvent is one or more of acetone, toluene, mineral oil, methyl acetate, 120# solvent oil, isooctane, isopropanol, chloroform, and methyl methacrylate, preferably, the organic solvent is one or more of 120# solvent oil, toluene, mineral oil, acetone, isooctane, and isopropanol, and more preferably, the organic solvent is 120# solvent oil, toluene, mineral oil, a mixed solvent of isooctane and isopropanol, or a mixed solvent of acetone and isopropanol;
(9) the mass percentage of the organic solvent in the additive is 69-79.5%; and
(10) the additive is composed of 20-30% of organocopper complex, 0.5-1% of plasticizer, and 69-79.5% of organic solvent.

3. A preparation method of a samarium-cobalt 2: 17 type magnet, **characterized by** comprising: mixing samarium-cobalt magnet alloy powder with the additive according to claim 1 or 2, shaping, sintering, and aging,
the mass percentage of Cu in the organocopper complex in the samarium-cobalt magnet alloy powder being 0.1-0.2%.

4. The preparation method of a samarium-cobalt 2: 17 type magnet according to claim 3, **characterized in that** the preparation method of a samarium-cobalt 2: 17 type magnet satisfies one or more of the following conditions:
(1) raw materials of the samarium-cobalt magnet alloy powder comprise Sm, Cu, Fe, Zr, and Co;
preferably, the mass percentage of Sm in the raw materials of the samarium-cobalt magnet alloy powder is 24-26% such as 24%, 25.5%, and 26%;
preferably, the mass percentage of Cu in the raw materials of the samarium-cobalt magnet alloy powder is 4-6% such as 4%, 5.5%, and 6%;
preferably, the mass percentage of Fe in the raw materials of the samarium-cobalt magnet alloy powder is 10-20% such as 10%, 17%, 19%, and 20%;
preferably, the mass percentage of Zr in the raw materials of the samarium-cobalt magnet alloy powder is 2.0-4% such as 2.0%, 3.5%, and 4%; and
preferably, the mass percentage of Co in the raw materials of the samarium-cobalt magnet alloy powder is 45-60% such as 46%, 48%, 51.5%, and 56%;
(2) the samarium-cobalt magnet alloy powder is obtained by melting and crushing the raw materials of the samarium-cobalt magnet alloy powder;
(3) the grain diameter D50 of the samarium-cobalt magnet alloy powder is 4-6 µm; and
(4) the samarium-cobalt magnet alloy powder is mixed with the additive, and the mixture is dried, shaped, sintered, and aged.

5. The preparation method of a samarium-cobalt 2: 17 type magnet according to claim 4, **characterized in that** the preparation method of a samarium-cobalt 2: 17 type magnet satisfies one or more of the following conditions:
(1) the samarium-cobalt magnet alloy powder is composed of 24% of Sm, 4% of Cu, 17% of Fe, 3.5% of Zr, and 51.5% of Co;
or, the samarium-cobalt magnet alloy powder is composed of 25.5% of Sm, 5.5% of Cu, 19% of Fe, 2% of Zr, and 48% of Co;
or, the samarium-cobalt magnet alloy powder is composed of 26% of Sm, 4% of Cu, 10% of Fe, 4% of Zr, and 56% of Co;
or, the samarium-cobalt magnet alloy powder is composed of 24% of Sm, 6% of Cu, 20% of Fe, 4% of Zr, and 46% of Co;
(2) the smelting is performed by melt-spinning, centrifugal casting or ingot casting;
(3) the crushing comprises coarse crushing, secondary crushing, and fine crushing, the coarse crushing is preferably Jaw crushing, the secondary crushing is preferably disc milling or crushing with an intermediate crusher, and the fine crushing is preferably jet milling or ball milling; and
(4) the drying is placing the powder in a dryer and drying at 80°C for 5-10 h, and the drying time is preferably 5 h, 6 h, 6.5 h, 7 h, 7.5 h, 8 h or 10 h.

6. The preparation method of a samarium-cobalt 2: 17 type magnet according to claim 3, **characterized in that** the preparation method of a samarium-cobalt 2: 17 type magnet satisfies one or more of the following conditions:
(1) the mass percentage of Cu in the organocopper complex in the samarium-cobalt magnet alloy powder is 0.1%, 0.12%, 0.14%, 0.16%, 0.18% or 0.2%;
(2) the additive is composed of 25% of copper naphthenate, 0.50% of epoxidized soybean oil, and 74.5% of 120# solvent oil, and the mass percentage of the additive in the samarium-cobalt magnet alloy powder is preferably 2.5%;
or, the additive is composed of 30% of copper oleate, 0.50% of epoxidized soybean oil, and 69.5% of 120# solvent oil, and the mass percentage of the additive in the samarium-cobalt magnet alloy powder is preferably 3.3%;
or, the additive is composed of 30% of copper hexadecanoate, 0.50% of dibutyl phthalate, and 69.5% of 120# solvent oil, and the mass percentage of the additive in the samarium-cobalt magnet alloy powder is preferably 3.6%;
or, the additive is composed of 27% of copper N,N-di-n-butyldithiocarbamate, 0.50% of dibutyl phthalate, and 72.5% of toluene, and the mass percentage of the additive in the samarium-cobalt magnet alloy powder is preferably 3.3%;
or, the additive is composed of 25% of copper dihexyldithiophosphate, 0.80% of epoxidized soybean oil, and 74.2% of toluene, and the mass percentage of the additive in the samarium-cobalt magnet alloy powder is preferably 3.4%;
or, the additive is composed of 22% of copper dibutyldithiophosphate, 0.80% of dioctyl phthalate, and 77.2% of mineral oil, and the mass percentage of the additive in the samarium-cobalt magnet alloy powder is preferably 2.4%;
or, the additive is composed of 23% of T541, 0.80% of dioctyl phthalate, and 76.2% of mineral oil, and the mass percentage of the additive in the samarium-cobalt magnet alloy powder is preferably 3.5%;
or, the additive is composed of 20% of copper acetylacetonate, 1% of epoxidized soybean oil, 40% of isooctane, and 39% of isopropanol, and the mass percentage of the additive in the samarium-cobalt magnet alloy powder is preferably 3.7%;
or, the additive is composed of 23% of copper acetoacetate, 1% of epoxidized soybean oil, 40% of acetone, and 36% of isopropanol, and the mass percentage of the additive in the samarium-cobalt magnet alloy powder is preferably 4.4%;
or, the additive is composed of 20% of copper hexadecanoate, 1% of epoxidized soybean oil, 40% of isooctane, and 39% of isopropanol, and the mass percentage of the additive in the samarium-cobalt magnet alloy powder is preferably 8.1%;
or, the additive is composed of 23% of copper oleate, 1% of epoxidized soybean oil, 40% of acetone, and 36% of isopropanol, and the mass percentage of the additive in the samarium-cobalt magnet alloy powder is preferably 8.7%.

7. The preparation method of a samarium-cobalt 2: 17 type magnet according to claim 3, **characterized in that** the preparation method of a samarium-cobalt 2: 17 type magnet satisfies one or more of the following conditions:
(1) the magnetic field strength B for shaping is 1.5-2 T;
(2) the sintering is performed in an inert atmosphere;
(3) the sintering temperature is 1200-1220°C such as 1200°C, 1210°C, 1215°C, and 1220°C;
(4) the sintering time is 1-5 h such as 1 h, 3 h, 4 h, and 5 h;
(5) solution treatment is performed after sintering,
preferably, the solution treatment temperature is 1140-1190°C such as 1140°C, 1150°C, 1160°C, and 1190°C;
preferably, the solution treatment time is 5-40 h such as 5 h, 20 h, 35 h, and 40 h, and
(6) the aging is keeping at 800-900°C for 5-20 h, cooling to 400°C, and keeping for 5-10 h,
preferably, the cooling is performed at a rate of 0.7°C/min.

## Patentansprüche

1. Verwendung eines Additivs, **dadurch gekennzeichnet, dass** es die folgenden Komponenten in Massenprozent umfasst: 20-30% eines Organokupferkomplexes, 0,5-1% eines Weichmachers und ein organisches Lösungsmittel, wobei die Summe der Massenprozentanteile der Komponenten 100% beträgt,
der Organokupferkomplex eine öllösliche Substanz ist, der Massenanteil von Cu im Organokupferkomplex größer als 10% ist, der Organokupferkomplex eine polare Gruppe und/oder eine Alkylkette mit mehr als 3 C-Atomen enthält,
bei der Herstellung eines Magneten des Typs Samarium-Kobalt 2:17.

2. Verwendung nach Anspruch 1, **dadurch gekennzeichnet, dass** das Additiv eine oder mehrere der folgenden Bedingungen erfüllt:
(1) die polare Gruppe in dem Organokupferkomplex ist eine oder mehrere von einer Hydroxylgruppe, einer Carboxylgruppe, einer Aminogruppe, einer Estergruppe und einer Amidgruppe;
(2) der Organokupferkomplex ist einer oder mehrere aus einem substituierten Kupfercarboxylatkomplex, einem Kupfercarboxylat-Derivat, einem Kupferthiophosphatkomplex, Kupferchinolin, Kupferhydroxychinolin, Kupferphthalat, Kupferthiodiazol, Kupferacetylacetonat und Kupferacetoacetat;
eine allgemeine Formel des substituierten Kupfercarboxylatkomplexes ist vorzugsweise [RCO₂]₂Cu, wobei R Alkyl, Alkinyl, Cyclo, Aryl oder Heteroaryl ist; vorzugsweise ist der substituierte Kupfercarboxylatkomplex einer oder mehrere von Kupferfettsäure mit 10 bis 22 Kohlenstoffatomen, Kupferstyrolmaleat, Kupferpicolinat, Kupfer-2-pyrazincarboxylat, Kupfer-2-ethylhexanoat, Kupfermethacrylat, Kupferthiophen-2-carboxylat, Kupfermethionin, und Kupfertartrat, und die Kupferfettsäure mit 10 bis 22 Kohlenstoffatomen ist vorzugsweise eine oder mehrere von Kupferoleat, Kupferlinoleat, Kupferstearat, Kupferrosinat, Kupferhexadecanoat, Kupferpalmitat und Kupfernaphthenat;
das Kupfercarboxylat-Derivat ist vorzugsweise ein Kupferthiocarboxylat-Derivat [R'CS₂]₂Cu oder ein Kupferselenocarboxylat-Derivat [R'CSe₂]₂Cu, wobei R' Alkyl und Alkylderivate umfasst; und vorzugsweise ist das Kupfercarboxylat-Derivat Kupfer-N,N-di-n-butyldithiocarbamat und/oder Kupfer-N,N-di-n-butyldiselenocarbamat;
der Kupferthiophosphatkomplex ist vorzugsweise ein Kupferkomplex eines Dialkyldithiophosphats, und eine allgemeine Formel des Kupferkomplexes des Dialkyldithiophosphats ist (RO)₂P(S)SHM, wobei R Alkyl oder Aryl ist und M einwertiges Kupfer und zweiwertiges Kupfer umfasst; und vorzugsweise ist der Kupferthiophosphatkomplex eines oder mehrere von Kupferdihexyldithiophosphat, Kupferdibutyldithiophosphat, kupferhaltigem Antioxidans T541, und kupferhaltigem Antioxidans T542;
(3) der Korndurchmesser des Organokupferkomplexes ist kleiner als 10 µm;
(4) der Massenanteil des Organokupferkomplexes im Additiv beträgt 20%, 22%, 23%, 25%, 27% oder 30%;
(6) der Weichmacher ist ein Phthalat und/oder epoxidiertes Sojabohnenöl, und vorzugsweise ist der Weichmacher eines oder mehrere von Dibutylphthalat, Dioctylphthalat und epoxidiertem Sojabohnenöl;
(7) der Massenprozentsatz des Weichmachers im Additiv beträgt 0,5%, 0,8% oder 1%;
(8) das organische Lösungsmittel ist eines oder mehrere aus Aceton, Toluol, Mineralöl, Methylacetat, 120#-Lösungsmittelöl, Isooctan, Isopropanol, Chloroform, und Methylmethacrylat, vorzugsweise ist das organische Lösungsmittel eines oder mehrere aus 120#-Lösungsmittelöl, Toluol, Mineralöl, Aceton, Isooctan, und Isopropanol, und mehr bevorzugt ist das organische Lösungsmittel 120#-Lösungsmittelöl, Toluol, Mineralöl, ein gemischtes Lösungsmittel aus Isooctan und Isopropanol oder ein gemischtes Lösungsmittel aus Aceton und Isopropanol;
(9) der Massenprozentsatz des organischen Lösungsmittels im Additiv beträgt 69-79,5%; und
(10) das Additiv besteht aus 20-30% Organokupferkomplex, 0,5-1% Weichmacher und 69-79,5% organischem Lösungsmittel.

3. Ein Verfahren zur Herstellung eines Magneten des Typs Samarium-Kobalt 2:17, **dadurch gekennzeichnet, dass** es umfasst: Mischen von Samarium-Kobalt-Magnet-Legierungspulver mit dem Additiv nach Anspruch 1 oder 2, Formen, Sintern und Altern,
wobei der Massenprozentsatz von Cu in dem Organokupferkomplex in dem Samarium-Kobalt-Magnet-Legierungspulver 0,1-0,2% beträgt.

4. Verfahren zur Herstellung eines Magneten des Typs Samarium-Kobalt 2:17 nach Anspruch 3, **dadurch gekennzeichnet, dass** das Verfahren zur Herstellung eines Magneten des Typs Samarium-Kobalt 2:17 eine oder mehrere der folgenden Bedingungen erfüllt:
(1) Die Rohmaterialien des Samarium-Kobalt-Magnet-Legierungspulvers umfassen Sm, Cu, Fe, Zr und Co;
vorzugsweise beträgt der Massenprozentsatz von Sm in den Rohmaterialien des Samarium-Kobalt-Magnet-Legierungspulvers 24-26%, wie z.B. 24%, 25,5% und 26%;
vorzugsweise beträgt der Massenprozentsatz von Cu in den Rohmaterialien des Samarium-Kobalt-Magnet-Legierungspulvers 4-6%, wie z.B. 4%, 5,5% und 6%;
vorzugsweise beträgt der Massenprozentsatz an Fe in den Rohmaterialien des Samarium-Kobalt-Magnet-Legierungspulvers 10-20%, wie z.B. 10%, 17%, 19% und 20%;
vorzugsweise beträgt der Massenprozentsatz von Zr in den Rohmaterialien des Samarium-Kobalt-Magnet-Legierungspulvers 2,0-4%, wie z.B. 2,0%, 3,5% und 4%; und
vorzugsweise beträgt der Massenprozentsatz von Co in den Rohmaterialien des Samarium-Kobalt-Magnet-Legierungspulvers 45-60%, wie z.B. 46%, 48%, 51,5%, und 56%;
(2) das Samarium-Kobalt-Magnet-Legierungspulver wird durch Schmelzen und Zerkleinern der Rohmaterialien des Samarium-Kobalt-Magnet-Legierungspulvers erhalten;
(3) der Korndurchmesser D50 des Samarium-Kobalt-Magnet-Legierungspulvers beträgt 4-6µm; und
(4) das Samarium-Kobalt-Magnet-Legierungspulver wird mit dem Additiv gemischt, und die Mischung wird getrocknet, geformt, gesintert und gealtert.

5. Verfahren zur Herstellung eines Magneten des Typs Samarium-Kobalt 2:17 nach Anspruch 4, **dadurch gekennzeichnet, dass** das Verfahren zur Herstellung eines Magneten des Typs Samarium-Kobalt 2:17 eine oder mehrere der folgenden Bedingungen erfüllt:
(1) das Samarium-Kobalt-Magnet-Legierungspulver besteht aus 24% Sm, 4% Cu, 17% Fe, 3,5% Zr und 51,5% Co;
oder das Samarium-Kobalt-Magnet-Legierungspulver besteht aus 25,5% Sm, 5,5% Cu, 19% Fe, 2% Zr und 48% Co;
oder das Samarium-Kobalt-Magnet-Legierungspulver besteht aus 26% Sm, 4% Cu, 10% Fe, 4% Zr und 56% Co;
oder das Samarium-Kobalt-Magnet-Legierungspulver besteht aus 24% Sm, 6% Cu, 20% Fe, 4% Zr und 46% Co;
(2) das Schmelzen wird durch Schmelzspinnen, Schleudergießen oder Barrengießen durchgeführt;
(3) die Zerkleinerung umfasst Grobzerkleinerung, Sekundärzerkleinerung und Feinzerkleinerung, wobei die Grobzerkleinerung vorzugsweise Backenbrechen ist, die Sekundärzerkleinerung vorzugsweise Scheibenvermahlung oder Zerkleinerung mit einem Zwischenbrecher ist und die Feinzerkleinerung vorzugsweise Strahlvermahlung oder Kugelvermahlung ist; und
(4) die Trocknung besteht darin, dass das Pulver in einen Trockner gegeben und bei 80°C für 5-10 h getrocknet wird, wobei die Trocknungszeit vorzugsweise 5h, 6h, 6,5h, 7h, 7,5h, 8h oder 10h beträgt.

6. Verfahren zur Herstellung eines Magneten des Typs Samarium-Kobalt 2: 17 nach Anspruch 3, **dadurch gekennzeichnet, dass** das Verfahren zur Herstellung eines Magneten des Typs Samarium-Kobalt 2: 17 eine oder mehrere der folgenden Bedingungen erfüllt:
(1) der Massenprozentsatz von Cu in dem Organokupferkomplex in dem Samarium-Kobalt-Magnet-Legierungspulver beträgt 0,1%, 0,12%, 0,14%, 0,16%, 0,18% oder 0,2%;
(2) das Additiv besteht aus 25% Kupfernaphthenat, 0,50% epoxidiertem Sojabohnenöl und 74,5% 120#-Lösungsmittelöl, und der Massenprozentsatz des Additivs in dem Samarium-Kobalt-Magnet-Legierungspulver beträgt vorzugsweise 2,5%;
oder das Additiv besteht aus 30% Kupferoleat, 0,50% epoxidiertem Sojabohnenöl und 69,5% 120#-Lösungsmittelöl, und der Massenprozentsatz des Additivs in dem Samarium-Kobalt-Magnet-Legierungspulver beträgt vorzugsweise 3,3%;
oder das Additiv besteht aus 30% Kupferhexadecanoat, 0,50% Dibutylphthalat und 69,5% 120#-Lösungsmittelöl, und der Massenprozentsatz des Additivs in dem Samarium-Kobalt-Magnet-Legierungspulver beträgt vorzugsweise 3,6%;
oder das Additiv besteht aus 27% Kupfer-N,N-di-n-butyldithiocarbamat, 0,50% Dibutylphthalat und 72,5% Toluol, und der Massenprozentsatz des Additivs in dem Samarium-Kobalt-Magnet-Legierungspulver beträgt vorzugsweise 3,3%;
oder das Additiv besteht aus 25% Kupferdihexyldithiophosphat, 0,80% epoxidiertem Sojabohnenöl und 74,2% Toluol, und der Massenprozentsatz des Additivs in dem Samarium-Kobalt-Magnet-Legierungspulver beträgt vorzugsweise 3,4%;
oder das Additiv besteht aus 22% Kupferdibutyldithiophosphat, 0,80% Dioctylphthalat und 77,2% Mineralöl, und der Massenprozentsatz des Additivs in dem Samarium-Kobalt-Magnet-Legierungspulver beträgt vorzugsweise 2,4%;
oder das Additiv besteht aus 23% T541, 0,80% Dioctylphthalat und 76,2% Mineralöl, und der Massenprozentsatz des Additivs in dem Samarium-Kobalt-Magnet-Legierungspulver beträgt vorzugsweise 3,5%;
oder das Additiv besteht aus 20% Kupferacetylacetonat, 1% epoxidiertem Sojabohnenöl, 40% Isooctan und 39% Isopropanol, und der Massenanteil des Additivs am Samarium-Kobalt-Magnet-Legierungspulver beträgt vorzugsweise 3,7%;
oder das Additiv besteht aus 23% Kupferacetoacetat, 1% epoxidiertem Sojabohnenöl, 40% Aceton und 36% Isopropanol, und der Massenprozentsatz des Additivs in dem Samarium-Kobalt-Magnet-Legierungspulver beträgt vorzugsweise 4,4%;
oder das Additiv besteht aus 20% Kupferhexadecanoat, 1% epoxidiertem Sojabohnenöl, 40% Isooctan und 39% Isopropanol, und der Massenprozentsatz des Additivs in dem Samarium-Kobalt-Magnet-Legierungspulver beträgt vorzugsweise 8,1%;
oder das Additiv besteht aus 23% Kupferoleat, 1% epoxidiertem Sojabohnenöl, 40% Aceton und 36% Isopropanol, und der Massenprozentsatz des Additivs in dem Samarium-Kobalt-Magnet-Legierungspulver beträgt vorzugsweise 8,7%.

7. Verfahren zur Herstellung eines Magneten des Typs Samarium-Kobalt 2:17 nach Anspruch 3, **dadurch gekennzeichnet, dass** das Verfahren zur Herstellung eines Magneten des Typs Samarium-Kobalt 2:17 eine oder mehrere der folgenden Bedingungen erfüllt:
(1) die magnetische Feldstärke B für die Formgebung beträgt 1,5-2T;
(2) das Sintern wird in einer inerten Atmosphäre durchgeführt
(3) die Sintertemperatur beträgt 1200-1220°C wie z.B. 1200°C, 1210°C, 1215°C und 1220°C;
(4) die Sinterzeit beträgt 1-5h, wie z.B. 1h, 3h, 4h und 5h;
(5) eine Lösungsbehandlung wird nach dem Sintern durchgeführt,
vorzugsweise beträgt die Temperatur der Lösungsbehandlung 1140-1190°C, wie z.B. 1140°C, 1150°C, 1160°C und 1190°C;
vorzugsweise beträgt die Lösungsbehandlungszeit 5-40h, wie z.B. 5h, 20h, 35h und 40h, und
(6) die Alterung erfolgt durch Halten bei 800-900°C für 5-20h, Abkühlen auf 400°C und Halten für 5-10h,
vorzugsweise wird die Kühlung mit einer Geschwindigkeit von 0,7°C/min durchgeführt.

## Revendications

1. Utilisation d'un additif, **caractérisée en ce qu'**elle comprend les composants suivants en pourcentage massique : 20 à 30% de complexe d'organo-cuivre, 0,5 à 1% de plastifiant, et un solvant organique, la somme des pourcentages massiques des composants étant de 100%,
le complexe d'organo-cuivre étant une substance soluble dans l'huile, le pourcentage massique de Cu dans le complexe d'organo-cuivre étant supérieur à 10%, le complexe d'organo-cuivre contenant un groupe polaire et/ou une chaîne alkyle ayant plus de 3 atomes de C,
dans la préparation d'un samarium-cobalt 2 : aimant de type 17.

2. Utilisation selon la revendication 1, **caractérisée en ce que** les additifs remplissent une ou plusieurs des conditions suivantes :
(1) le groupe polaire dans le complexe d'organo-cuivre est un ou plusieurs parmi un groupe hydroxyle, un groupe carboxyle, un groupe amino, un groupe ester et un groupe amide ;
(2) le complexe d'organo-cuivre est un ou plusieurs parmi un complexe de carboxylate de cuivre substitué, un dérivé de carboxylate de cuivre, un complexe de thiophosphate de cuivre, la quinoléine de cuivre, l'hydroxyquinoléine de cuivre, le phtalate de cuivre, le thiodiazole de cuivre, l'acétylacétonate de cuivre et l'acétoacétate de cuivre ;
une formule générale du complexe de carboxylate de cuivre substitué est de préférence [RCO₂]₂Cu, où, R est alkyle, alcynyle, cyclo, aryle ou hétéroaryle ; de préférence, le complexe de carboxylate de cuivre substitué est un ou plusieurs parmi le cuivre d'acide gras ayant 10 à 22 atomes de carbone, le maléate de styrène de cuivre, le picolinate de cuivre, le 2-pyrazinecarboxylate de cuivre, le 2-éthylhexanoate de cuivre, le méthacrylate de cuivre, le thiophène-2-carboxylate de cuivre, la méthionine de cuivre et le tartrate de cuivre, et le cuivre d'acide gras ayant 10 à 22 atomes de carbone est de préférence un ou plusieurs parmi l'oléate de cuivre, le linoléate de cuivre, le stéarate de cuivre, le rosinate de cuivre, l'hexadécanoate de cuivre, le palmitate de cuivre et le naphténate de cuivre ;
le dérivé de carboxylate de cuivre est de préférence un dérivé de thiocarboxylate de cuivre [R'CS₂]₂Cu ou un dérivé de sélénocarboxylate de cuivre [R'CSe₂]₂Cu, où, R' comprend un alkyle et des dérivés d'alkyle ; et de préférence, le dérivé de carboxylate de cuivre est le N,N-di-n-butyldithiocarbamate de cuivre et/ou le N, N-di-n-butyldisélénocarbamate de cuivre ;
le complexe de thiophosphate de cuivre est de préférence un complexe de cuivre d'un dialkyldithiophosphate, et une formule générale du complexe de cuivre du dialkyldithiophosphate est (RO)₂P(S)SHM, où, R est un alkyle ou un aryle, et M comprend du cuivre monovalent et du cuivre divalent ; et de préférence, le complexe de thiophosphate de cuivre est un ou plusieurs parmi le dihexyldithiophosphate de cuivre, le dibutyldithiophosphate de cuivre, l'antioxydant contenant du cuivre T541 et l'antioxydant contenant du cuivre T542 ;
(3) le diamètre de grain du complexe d'organo-cuivre est inférieur à 10 µm ;
(4) le pourcentage massique du complexe d'organo-cuivre dans l'additif est de 20%, 22%, 23%, 25%, 27% ou 30% ;
(6) le plastifiant est un phtalate et/ou une huile de soja époxydée, et de préférence, le plastifiant est un ou plusieurs parmi le phtalate de dibutyle, le phtalate de dioctyle et l'huile de soja époxydée ;
(7) le pourcentage massique du plastifiant dans l'additif est de 0,5%, 0,8% ou 1% ;
(8) le solvant organique est un ou plusieurs parmi l'acétone, le toluène, l'huile minérale, l'acétate de méthyle, l'huile de solvant 120#, l'isooctane, l'isopropanol, le chloroforme et le méthacrylate de méthyle, de préférence, le solvant organique est un ou plusieurs parmi l'huile de solvant 120#, le toluène, l'huile minérale, l'acétone, l'isooctane et l'isopropanol, et plus préférablement, le solvant organique est l'huile de solvant 120#, le toluène, l'huile minérale, un solvant mixte d'isooctane et d'isopropanol, ou un solvant mixte d'acétone et d'isopropanol ;
(9) le pourcentage massique du solvant organique dans l'additif est de 69 à 79,5% ; et
(10) l'additif est composé de 20-30% de complexe d'organo-cuivre, 0,5 à 1% de plastifiant et 69 à 79,5% de solvant organique.

3. Procédé de préparation d'un samarium-cobalt 2 : aimant de type 17, **caractérisé en ce qu'**il comprend : le mélange de la poudre d'alliage magnétique de samarium-cobalt avec l'additif selon la revendication 1 ou 2, la mise en forme, le frittage et le vieillissement,
le pourcentage massique de Cu dans le complexe d'organo-cuivre dans la poudre d'alliage magnétique de samarium-cobalt étant de 0,1 à 0,2 %.

4. Procédé de préparation d'un samarium-cobalt 2 : aimant de type 17 selon la revendication 3, **caractérisé en ce que** le procédé de préparation d'un samarium-cobalt 2 : l'aimant de type 17 remplit une ou plusieurs des conditions suivantes :
(1) les matières premières de la poudre d'alliage magnétique de samarium-cobalt comprennent Sm, Cu, Fe, Zr et Co ;
de préférence, le pourcentage massique de Sm dans les matières premières de la poudre d'alliage magnétique de samarium-cobalt est de 24 à 26%, à savoir 24%, 25,5% et 26% ;
de préférence, le pourcentage massique de Cu dans les matières premières de la poudre d'alliage magnétique de samarium-cobalt est de 4 à 6%, à savoir 4%, 5,5% et 6% ;
de préférence, le pourcentage massique de Fe dans les matières premières de la poudre d'alliage magnétique de samarium-cobalt est de 10 à 20%, à savoir 10%, 17%, 19% et 20% ;
de préférence, le pourcentage massique de Zr dans les matières premières de la poudre d'alliage magnétique de samarium-cobalt est de 2,0 à 4%, à savoir 2,0%, 3,5% et 4% ; et
de préférence, le pourcentage massique de Co dans les matières premières de la poudre d'alliage magnétique de samarium-cobalt est de 45 à 60%, à savoir 46%, 48%, 51,5% et 56% ;
(2) la poudre d'alliage magnétique de samarium-cobalt est obtenue par fusion et broyage des matières premières de la poudre d'alliage magnétique de samarium-cobalt ;
(3) le diamètre de grain D50 de la poudre d'alliage magnétique de samarium-cobalt est de 4 à 6 µm ; et
(4) la poudre d'alliage magnétique de samarium-cobalt est mélangée à l'additif, et le mélange est séché, mis en forme, fritté et vieilli.

5. Procédé de préparation d'un samarium-cobalt 2 : aimant de type 17 selon la revendication 4, **caractérisé en ce que** le procédé de préparation d'un samarium-cobalt 2 : l'aimant de type 17 remplit une ou plusieurs des conditions suivantes :
(1) la poudre d'alliage magnétique de samarium-cobalt est composée de 24% de Sm, 4% de Cu, 17% de Fe, 3,5% de Zr et 51,5% de Co ;
ou, la poudre d'alliage magnétique de samarium-cobalt est composée de 25,5% de Sm, 5,5% de Cu, 19% de Fe, 2% de Zr et 48% de Co ;
ou, la poudre d'alliage magnétique de samarium-cobalt est composée de 26% de Sm, 4% de Cu, 10% de Fe, 4% de Zr et 56% de Co ;
ou, la poudre d'alliage magnétique de samarium-cobalt est composée de 24% de Sm, 6% de Cu, 20% de Fe, 4% de Zr et 46% de Co ;
(2) la fusion est effectuée par filage à chaud, moulage par centrifugation ou coulée en lingotière ;
(3) le broyage comprend un broyage grossier, un broyage secondaire et un broyage fin, le broyage grossier est de préférence un broyage à mâchoires, le broyage secondaire est de préférence un broyage à disque ou un broyage avec un broyeur intermédiaire, et le broyage fin est de préférence une désintégration à jet ou un broyage à boulets ; et
(4) le séchage consiste à placer la poudre dans un séchoir et à la sécher à 80 °C pendant 5 à 10 h, et le temps de séchage est de préférence de 5 h, 6 h, 6,5 h, 7 h, 7,5 h, 8 h ou 10 h.

6. Procédé de préparation d'un samarium-cobalt 2 : aimant de type 17 selon la revendication 3, **caractérisé en ce que** le procédé de préparation d'un samarium-cobalt 2 : l'aimant de type 17 remplit une ou plusieurs des conditions suivantes :
(1) le pourcentage massique de Cu dans le complexe d'organo-cuivre dans la poudre d'alliage magnétique de samarium-cobalt est de 0,1%, 0,12%, 0,14%, 0,16%, 0,18% ou 0,2% ;
(2) l'additif est composé de 25% de naphténate de cuivre, 0,50% d'huile de soja époxydée et 74,5% d'huile de solvant 120#, et le pourcentage massique de l'additif dans la poudre d'alliage magnétique de samarium-cobalt est de préférence de 2,5% ;
ou, l'additif est composé de 30% d'oléate de cuivre, 0,50% d'huile de soja époxydée et 69,5% d'huile de solvant 120#, et le pourcentage massique de l'additif dans la poudre d'alliage magnétique de samarium-cobalt est de préférence de 3,3% ;
ou, l'additif est composé de 30% d'hexadécanoate de cuivre, 0,50% de phtalate de dibutyle et 69,5% d'huile de solvant 120#, et le pourcentage massique de l'additif dans la poudre d'alliage magnétique de samarium-cobalt est de préférence de 3,6 % ;
ou, l'additif est composé de 27% de N,N-di-n-butyldithiocarbamate de cuivre, de 0,50% de phtalate de dibutyle et de 72,5% de toluène, et le pourcentage massique de l'additif dans la poudre d'alliage magnétique de samarium-cobalt est de préférence de 3,3% ;
ou, l'additif est composé de 25% de dihexyldithiophosphate de cuivre, 0,80% d'huile de soja époxydée et 74,2% de toluène, et le pourcentage massique de l'additif dans la poudre d'alliage magnétique samarium-cobalt est de préférence de 3,4% ;
ou, l'additif est composé de 22% de dibutyldithiophosphate de cuivre, 0,80% de phtalate de dioctyle et 77,2% d'huile minérale, et le pourcentage massique de l'additif dans la poudre d'alliage magnétique de samarium-cobalt est de préférence de 2,4% ;
ou, l'additif est composé de 23% de T541, 0,80% de phtalate de dioctyle et 76,2% d'huile minérale, et le pourcentage massique de l'additif dans la poudre d'alliage magnétique de samarium-cobalt est de préférence de 3,5% ;
ou, l'additif est composé de 20% d'acétylacétonate de cuivre, 1% d'huile de soja époxydée, 40% d'isooctane et 39% d'isopropanol, et le pourcentage massique de l'additif dans la poudre d'alliage magnétique de samarium-cobalt est de préférence de 3,7% ;
ou, l'additif est composé de 23% d'acétoacétate de cuivre, 1 % d'huile de soja époxydée, 40% d'acétone et 36% d'isopropanol, et le pourcentage massique de l'additif dans la poudre d'alliage magnétique de samarium-cobalt est de préférence de 4,4% ;
ou, l'additif est composé de 20% d'hexadécanoate de cuivre, 1% d'huile de soja époxydée, 40% d'isooctane et 39% d'isopropanol, et le pourcentage massique de l'additif dans la poudre d'alliage magnétique de samarium-cobalt est de préférence de 8,1% ;
ou, l'additif est composé de 23% d'oléate de cuivre, 1% d'huile de soja époxydée, 40% d'acétone et 36% d'isopropanol, et le pourcentage massique de l'additif dans la poudre d'alliage magnétique de samarium-cobalt est de préférence de 8,7%.

7. Procédé de préparation d'un samarium-cobalt 2 : aimant de type 17 selon la revendication 3, **caractérisé en ce que** le procédé de préparation d'un samarium-cobalt 2 : l'aimant de type 17 remplit une ou plusieurs des conditions suivantes :
(1) l'intensité du champ magnétique B pour la mise en forme est de 1,5 à 2 T ;
(2) le frittage est effectué sous une atmosphère inerte ;
(3) la température de frittage est de 1200 à 1220 °C, à savoir 1200 °C, 1210 °C, 1215 °C et 1220 °C ;
(4) le temps de frittage est de 1 à 5 h, à savoir 1 h, 3 h, 4 h et 5 h ;
(5) le traitement de solution est effectué après le frittage,
de préférence, la température de traitement de solution est de 1140 à 1190 °C, à savoir 1140 °C, 1150 °C, 1160 °C et 1190 °C ;
de préférence, le temps de traitement de solution est de 5 à 40 h, à savoir 5 h, 20 h, 35 h et 40 h, et
(6) le vieillissement se maintient de 800 à 900°C pendant 5 à 20 h, le refroidissement à 400°C et le maintien pendant 5 à 10 h,
de préférence, le refroidissement est effectué à une vitesse de 0,7 °C/min.
